

## UNITED STATES PATENT OFFICE

ROTHE WEIGEL, OF NASHVILLE, TENNESSEE, ASSIGNOR TO VICTOR CHEMICAL WORKS,  
A CORPORATION OF ILLINOIS

## PRODUCTION OF PHOSPHORUS

No Drawing.

Application filed June 8, 1931. Serial No. 543,028.

The present invention relates to improvements in the production of phosphorus and phosphorus compounds by volatilization processes, and more particularly to the production of phosphorus and phosphorus compounds from natural phosphate minerals in the blast furnace processes.

It has hitherto been proposed, in the production of phosphorus and phosphorus compounds, to grind the natural phosphate mineral, for example, a phosphate rock and form it into briquettes with carbonaceous material and silicious material, the carbonaceous material being provided in a proportion such as to give the resulting briquetted mass a carbon content substantially in excess of that theoretically required in the reduction reaction and the proportion of silicious material being such as to provide all or at least part of that necessary for the reaction. In carrying out the operation in the blast furnace, the briquettes thus produced have been charged into the furnace, together with coke in sufficient quantity to provide the fuel requirements for the operation of the furnace with usually some excess thereover and, when necessary, additional silicious material for the reaction, suitably in the form of silica pebble. In operating in this manner, for example, the ratio of the fuel coke supplied relative to the briquettes and silica has ordinarily varied, say from 0.730:1 to 0.750:1. By employing the ground phosphate mineral in briquetted form, it is possible to employ run-of-mine and fine phosphate rock and other phosphate minerals and to secure a uniform composition of feed.

It has now been found that a marked improvement in operating conditions of a volatilization furnace operating upon a briquetted charge may be effected by reducing the content of carbonaceous material incorporated in the briquettes with the phosphate rock or other phosphate mineral to substantially less than that required theoretically in the reduction reaction, and preferably to form 25 to 75% of the theoretical proportion. The proportion of carbon to  $P_2O_5$  theoretically required for the reaction is 0.422:1, and in operating in accordance with the present in-

vention, it is preferred to reduce its ratio substantially, preferably to not higher than 0.306:1. In a typical operation, I have employed a ratio of carbon to  $P_2O_5$  of approximately 0.153:1.

The following example illustrates an operation in accordance with the present invention, it being understood, however, that the scope of the invention is not limited by the specific details of the example as herein set forth.

The phosphate rock employed is a run-of-mine rock showing, on the usual proximate analysis, 3.35% moisture; 25.03%  $P_2O_5$  and 33.65% CaO. The phosphate rock is ground to suitable fineness say, below 20 mesh and preferably from 30-40 mesh, and is formed into briquettes with the desired carbonaceous material, for example, bituminous coal, the silicious material in the desired proportions (or if a highly silicious phosphate rock is used, extra silicious material may be omitted), a suitable organic binder such as sulfite liquor, molasses or the like being employed. After briquetting, the briquettes are dried. In the case of the phosphate rock above described, which has a high silica content, the briquettes may be formed from a mixture containing 92.25% of the phosphate rock, 6% of coal and 1.75% of a sulfite liquor containing 50% solids. The coal employed contains about 62% carbon and the briquettes produced, after drying, have the following composition:

|          |        |
|----------|--------|
| Moisture | 0.99%  |
| $P_2O_5$ | 24.29% |
| $SiO_2$  | 21.62% |
| CaO      | 32.41% |
| Carbon   | 3.71%  |

The proportion of carbon contained in the briquettes is slightly more than 36% of that theoretically required for the reduction reaction.

The blast furnace, which is started with coke and slag, is fed with these briquettes together with additional silica, when necessary, the latter preferably in pebble form, and with the requisite coke for fuel. The proportions of silicious material either incorpo-

55

60

65

70

75

80

85

90

100

rated directly in the briquettes or that in the briquettes together with the added silica, is calculated as in ordinary blast furnace practice to give a readily fusible fluid slag; for example, to maintain a ratio of  $\text{SiO}_2$  to  $\text{CaO}$  of 0.8:1, or suitably within the range of from 0.6:1 to 1.2:1. With briquettes of the constant average composition above set forth, in a typical operation, the ratio of briquettes and added silicious material to fuel coke may be in the proportion of 100 parts of briquettes and 4 parts of added silica to 70.3 parts of coke. It will be understood, of course, that the silicious material may be incorporated in the briquettes if desired, and that the proportions of the various constituents will vary, as in ordinary blast furnace practice, in accordance with the operating conditions desired and the relative proportions of lime to silica desired in the slag, and that the proportions above given merely illustrate a typical operation in accordance with the invention.

By operating in accordance with the present invention, with the proportion of carbonaceous material incorporated in briquettes of constant average composition markedly less than that required for theoretical reduction of the phosphate, it has been found that certain marked improvements in the operation of the blast furnace are effected. The proportion of fuel coke or carbonaceous material extraneous to the briquettes required for the operation of the furnace, which is controlled to secure the desired hearth temperature, is not increased; on the contrary, it has been found that it may be reduced as much as 4 to 8% or even 10%. The desired high hearth temperatures, say about  $1600^{\circ}$  C. are more easily maintained, with a more effective liberation and volatilization of the phosphorus, an increased yield, and a reduction of the phosphate content of the slag. Particularly marked are the reductions in quantity of very fine flue dust or fume carried by the gases from the blast furnace and the reduction in accumulations of infusible material in the hearth zone of the furnace.

In carrying out the present invention, it is found desirable that some carbonaceous material be incorporated in the briquettes of constant average composition which are used in charging the furnace, in proportion at least 15% of the theoretical requirements, based upon the  $\text{P}_2\text{O}_5$  present. While coke may be employed for the purpose, it is preferred that a carbonaceous material containing volatilizable hydrocarbons be employed, such as anthracite coal or preferably bituminous coal, the proportion of the carbonaceous material being such as to provide the desired quantity of fixed carbon in the briquette. It is preferred that the proportion of carbon incorporated in the briquettes shall not exceed 75% of the theoretical, and in general 30 to

40% of the theoretical requirements is employed.

I claim:

1. The method of producing phosphorus in a volatilization furnace which comprises commingling phosphorus-containing mineral with a proportion of carbonaceous material less than that required for reduction of its phosphorus content and forming coherent briquettes of constant average composition therefrom, charging such briquettes into the furnace to pass into the volatilization zone therein, and maintaining a temperature in said furnace to liberate phosphorus and form a molten slag. 70  
75

2. The method of producing phosphorus in a volatilization furnace which comprises commingling phosphorus-containing mineral, silicious material, and a proportion of carbonaceous material less than that required for reduction of the phosphorus content of the mineral, forming coherent briquettes of constant average composition from the mixture, and charging such briquettes with additional carbonaceous material into the furnace to pass into the volatilization zone therein, and maintaining a temperature in said furnace to liberate phosphorus and form a molten slag. 80  
85

3. The method of producing phosphorus in a blast furnace which comprises commingling ground phosphate mineral and silicious material with carbonaceous material in proportion substantially less than that required for reduction of the phosphorus, forming coherent briquettes of the mixture, and charging such briquettes into the furnace with added carbonaceous material required to maintain, by combustion, the desired temperature in the furnace, and maintaining a temperature in the furnace by combustion of said fuel to liberate phosphorus and form a molten slag. 95  
100

4. The method of producing phosphorus in a blast furnace which comprises commingling ground phosphate rock with carbonaceous material containing volatile hydrocarbon constituents, the proportion of carbonaceous material being less than that required for reduction of the phosphorus, forming coherent briquettes of the mixture, charging said briquettes together with carbon for fuel into the furnace to pass therethrough, and maintaining a temperature in the furnace by combustion of said fuel carbon to liberate phosphorus and form a molten slag. 110  
115  
120

5. The method of producing phosphorus in a blast furnace which comprises commingling ground phosphate rock with carbonaceous material in a proportion from 15 to 75% of that required for reduction of the phosphorus, forming briquettes of said mixture, charging such briquettes into the furnace together with carbonaceous material in amount required 125  
130

for fuel and supplying silicious material in the furnace in proportion to supply the requirements for slag of desired composition, said materials passing through the furnace, and maintaining a temperature in the furnace by combustion of the carbonaceous material therein to liberate phosphorus and form a molten slag.

6. The method of producing phosphorus  
10 in a blast furnace which comprises commingling ground phosphate rock with carbonaceous material in a proportion from 30 to 40% of that required for reduction of the phosphorus, forming briquettes of said mixture, charging such briquettes into the furnace together with carbonaceous material in amount required for fuel and supplying silicious material in the furnace in proportion to supply the requirements for slag of  
15 desired composition, said materials passing through the furnace, and maintaining a temperature in the furnace by combustion of the carbonaceous material therein to liberate phosphorus and form a molten slag.

20 7. A briquette for use in a phosphorus volatilization furnace, said briquette comprising phosphate mineral and carbonaceous material to supply carbon in proportion from 15 to 75% of that required for reduction of  
25 the phosphorus of the mineral.

8. A briquette for use in a phosphorus volatilization furnace, said briquette comprising phosphate mineral and carbonaceous material containing volatile hydrocarbon  
30 constituents, said carbonaceous material being present in proportion to supply carbon to the extent of 15 to 75% of that required for reduction of the phosphorus of the mineral.

35 9. A briquette for use in a phosphorus volatilization furnace, said briquette comprising phosphate mineral and carbonaceous material containing volatile hydrocarbon constituents, said carbonaceous material being present in proportion to supply carbon to  
40 the extent of 30 to 40% of that required for reduction of the phosphorus of the mineral.

45 ROTHE WEIGEL.

50

55

60

65